

# UNITED STATES PATENT OFFICE.

SAMPSON GAMGEE, OF BIRMINGHAM, COUNTY OF WARWICK, ASSIGNOR  
TO WILLIAM BRADBURY ROBINSON, OF WHEAT BRIDGE MILLS, NEW  
BRAMPTON, ENGLAND.

## MANUFACTURE OF FABRICS FOR SURGICAL AND MEDICAL DRESSING.

SPECIFICATION forming part of Letters Patent No. 282,624, dated August 7, 1883.

Application filed June 30, 1883. (No specimens.)

*To all whom it may concern:*

Be it known that I, SAMPSON GAMGEE, a subject of the Queen of Great Britain, residing at 22 Broad Street, Birmingham, in the 5 county of Warwick, England, have invented certain new and useful Improvements in the Manufacture of Fabrics for Surgical and Medical Dressings, and the Manufacture of Surgical Splints and Supports; and I do hereby declare that the following is a full, clear, and 10 exact description of the invention, which will enable others skilled in the art to which it appertains to make and use the same.

This invention has for its object improvements in the manufacture of fabrics for surgical and medical dressings, and in the manufacture of surgical splints and supports.

I produce a fabric for surgical and medical dressings from thoroughly-bleached cotton. I 15 inclose a sheet of this fiber between two muslin fabrics. These fabrics are of an open nature, thoroughly bleached, and freed from dressing, and the fiber is compressed between them. The compound fabric may conveniently be 20 made of different thicknesses—say thin, medium, and thick—and varying from four ounces in weight to ten ounces in weight to the square yard. This absorbent cotton-wool tissue is calculated to prove of very great service in medical and surgical practice. The perfect smoothness and elasticity specially fit it for application 25 to inflamed parts, while its perfectly even surface specially adapts it to be a medium for equable pressure. It never becomes knotty 30 or lumpy, like ordinary cotton-wool, and its powerful absorbing and antiseptic properties prevent the retention and decomposition of skin and wound secretions.

Another part of the invention relates to 35 splints and surgical supports.

I have ascertained that the absorbent wool-tissue above described becomes immediately impregnated with a liquid mixture of plaster-of-paris on being dipped into it. I apply this 40 fact to the manufacture of splints and supports as follows: I surround a form to which the splint or support is to be molded, or it may be an actual hand or limb, with a layer of absorbent wool tissue, and outside this I mold 45 another layer of the same tissue, previously

soaked in plaster-of-paris cream. This cream is made by sprinkling in water perfectly fresh and powdered plaster-of-paris. I stir with a metal spoon, and continue sprinkling the powder until the liquid acquires the consistence 55 of rich cream or thin batter. The tissue, on being pressed into the liquid, very quickly becomes completely saturated. It requires to be lightly squeezed to expel redundant cream, and is then fit to be smoothly applied over the 60 layer of dry tissue with which the part has previously been covered. Bandaging with a white, soft, absorbent roller, the plaster covering is molded accurately and without constriction. It rapidly dries and hardens; but this 65 process may be hastened by unrolling the bandage, carefully removing the mold, and holding it for a few minutes before the fire. It can then be reapplied, and it will be found that while the outer shell is hard the inner 70 lining retains all the softness and elasticity of the original tissue. The splints may be cut to any shape, adapted to any surfaces, and almost instantly solidified. Given a case of fracture of the pelvis, spine, or ribs, a layer of 75 the dry absorbent tissue having been rolled round the patient, one or two more layers bandaged outside it, after having been previously soaked in plaster cream, result in the construction of a solid shell, with which fragments are held motionless and harmless. By cutting strips of the tissue and soaking them in plaster-cream, any joint may be immobilized 80 by a plaster-and-bandage brace, or lattice-work. If desired, gum-arabic, starch, or dextrine may be added to the plaster-cream.

Skill in making the molds may be readily acquired by anyone cutting pieces of the tissue, soaking them in plaster-cream, and molding them with the hands upon a form. However unequal the surface, a perfect mold can be taken. It quickly solidifies, and can be readily taken off. One effect resulting from impregnation 85 of the gauze and cotton fiber with plaster is that the resulting mold is not brittle, but on the contrary so tough that it is almost impossible to break or tear it. Since the molds and splints can be made and removed in sections, the usual difficulty in opening and removing a plaster-of-paris case is entirely obviated.

An excellent result is obtained when a mixture of dextrine and plaster-of-paris is employed—say in the proportion of three parts of dextrine to eight parts of plaster and twelve parts of water. The mixture is made as already described, except that the solution of dextrine is employed in the place of water. The tissue, having been dipped in the compound and applied in the manner explained above, rapidly sets, and so very light, strong, and flexible splints and supports may be produced. These splints and supports can be afterward softened, if desired, by immersing them in hot water. They can then be bent to another form, which they will retain on cooling. Gum-arabic or starch can be used in place of dextrine, but less advantageously, and other like materials may be employed as a substitute for plaster-of-paris.

My compound fabric or tissue may also very advantageously be used in combination with paraffine in the manufacture of splints and supports. The fabric or tissue is dipped in melted paraffine, removed and slightly pressed to remove excess, and applied to the form or part. Cold water may be poured over to hasten the hardening. The splints and supports may also be made from paraffine-saturated fabric previously prepared, and again softened by heat when required for use. Strips of thin deal-veneer, in parallel lines or intersecting lattice-work fashion between two layers of paraffined absorbent tissue, make an exceedingly strong splintage. This material may be cut to any size with an ordinary pair of scissors, molded to any shape after exposure to slight heat, and rapidly solidified on being sponged with cold water. Incorporated, as the paraffine is, with the cotton and gauze, the resulting tissue is not in the least brittle; nor, indeed, are the molds made with the plaster-of-paris cream.

The paraffine and plaster splintage may be perforated to facilitate drainage, and that made with paraffine has the further advantage of being especially well adapted for the application of pressure. Besides its well-known intrinsic antiseptic properties, paraffine readily takes up borax and other anti-putrescent agents.

Having thus described the nature of my said invention and the manner of performing the same, I would have it understood that I claim—

1. My improved compound fabric, consisting of thoroughly-bleached absorbent cotton compressed between two thoroughly-bleached muslin fabrics free from stiffening, substantially as described.

2. The means for producing my compound fabric by accumulating the fleeces from a series of carding-engines and passing and compressing the same between fabrics drawn continuously from rollers, substantially as described.

3. The manufacture of surgical splints and supports from my compound fabric saturated with plaster-of-paris or other material, and molded on a form upon which it sets and hardens, substantially as described.

4. My compound fabric saturated with glucose, gum-arabic, or starch, (mixed preferably with plaster-of-paris,) and the manufacture of surgical splints or supports therefrom, substantially as described.

5. My compound fabric saturated with paraffine, and the manufacture of surgical splints or supports therefrom, substantially as described.

SAMPSON GAMGEE.

Witnesses:

J. EDWD. NEWMAN,

H. DICKIN,

*Notary's Clerks, Birmingham.*